# EUROPEAN PATENT APPLICATION

(11) **EP 0 466 307 A1**
(43) Date of publication of application: **15.01.1992**
(21) Application number: 91304307.1
(22) Date of filing: 14.05.1991
(51) Int. Cl.: C10M 111/04

(54) **Synthetic lubricant base stocks**

(30) Priority: 12.06.1990 US 536906; 28.06.1990 US 545260
(71) Applicant: TEXACO CHEMICAL COMPANY, Houston, Texas 77056 (US)
(72) Inventor: Sanderson, John Ronald, Leander, Texas 78641 (US); Marquis, Edward Thomas, Austin, Texas 78758 (US)
(74) Representative: Brock, Peter William

(57) **Abstract**

Synthetic lubricant base stocks comprise oligomers prepared by reacting an olefin composition comprising a linear olefin having from 10 to 24 carbon atoms, in the presence of an acid montmorillonite clay and of anisole, diphenyl ether or diphenyl, thereby providing products which additionally contain an alkyl-substituted diphenyl, diphenyl ether or anisole having the formula:
wherein R¹ is a group of the formula
and where R², R³, R⁴, R⁵ R⁶ and R⁷ are each H or an alkyl group having 1 to 24 carbon atoms, provided that at least one of R², R³, R⁴, R⁵, R⁶ and R⁷ is an alkyl group containing from 10 to 24 carbon atoms, R¹¹ is an alkyl group having 1 to 10 carbon atoms; R² is an alkyl group having 10 to 24 carbon atoms; and R³ and R⁴ are each H or an alkyl group having up to 10 carbon atoms. The resulting product may be completely or partially hydrogenated.

## Description

The invention relates to synthetic lubricant base stocks, and more particularly to synthetic lubricant base stocks having a good viscosity. Some of these also exhibit a low pour point.

Synthetic lubricants prepared from man-made base stocks have uniform molecular structures and, therefore, well-defined properties that can be tailored to specific applications. Mineral oil base stocks, on the other hand, are prepared from crude oil and are complex mixtures of naturally occurring hydrocarbons. The greater uniformity of synthetic lubricants generally results in superior performance properties. For example, synthetic lubricants have excellent thermal stability. As automobile engines are reduced in size to save weight and fuel, they run at higher temperatures, and therefore require a more thermally stable oil. Because lubricants made from synthetic base stocks have such properties as excellent oxidative/thermal stability, very low volatility, and good viscosity indices over a wide range of temperatures, they offer better lubrication and permit longer drain intervals, with less oil vaporization loss between oil changes.

Synthetic base stocks may be prepared by oligomerizing internal and alpha-olefin monomers to form a mixture of dimers, trimers, tetramers, and pentamers, with minimal amounts of higher oligomers. The unsaturated oligomer products are then hydrogenated to improve their oxidative stability, with little change in other properties. The resulting synthetic base stocks have uniform isoparaffinic hydrocarbon structures, similar to those of high quality paraffinic mineral base stocks, but have the superior properties mentioned because of their greater uniformity.

Synthetic base stocks are produced in a broad range of viscosity grades. It is common practice to classify the base stocks by their viscosities, measured in centistokes (cSt) at 100°C. Those base stocks with viscosities less than or equal to 4 cSt are commonly referred to as "low viscosity" base stocks, whereas base stocks having a viscosity of 40 to 100 cSt are commonly referred to as "high viscosity" base stocks. Base stocks having a viscosity of 4 to 8 cSt are referred to as "medium viscosity" base stocks. The low viscosity base stocks generally are recommended for low temperature applications. Base stocks for higher temperature applications, such as motor oils, automatic transmission fluids, turbine lubricants, and other industrial lubricants, generally require higher viscosities, such as those provided by medium viscosity base stocks (i.e. 4 to 8 cSt grades). High viscosity base stocks are used in gear oils and as blending stocks.

The viscosity of the base stocks generally is determined by the length of the oligomer molecules formed during the oligomerization reaction. The degree of oligomerization is affected by the catalyst and reaction conditions employed during the oligomerization reaction. The length of the carbon chain of the monomer starting material also has a direct influence on the properties of the oligomer products. Fluids prepared from short-chain monomers tend to have low pour points and moderately low viscosity indices, whereas fluids prepared from long-chain monomers tend to have moderately low pour points and higher viscosity indices. Oligomers prepared from long-chain monomers are generally more suitable for use as medium viscosity synthetic lubricant base stocks than those prepared from shorter-chain monomers.

One known approach to oligomerizing long-chain olefins to prepare synthetic lubricant base stocks is to contact the olefin with boron trifluoride, together with a promoter, at a reaction temperature sufficient to effect oligomerization of the olefin, as described in US-A-4400565, -4420646, -4420647 and -4434308. Boron trifluoride gas (BF₃) is however a pulmonary irritant, and breathing the gas, or fumes formed by hydration of the gas with atmospheric moisture, poses hazards preferably avoided. Additionally, the disposal/neutralization of BF₃ raises environmental concerns. Thus, a method for oligomerizing long-chain olefins using a non-hazardous, non-polluting catalyst would be a substantial improvement in the art.

Kuliev et al. "Preparation of High-Viscosity Synthetic Lubricants Using an Aluminosilicate Catalyst" Institute of Petrochemical Processes of the Academy of Sciences of the Azerbaidzhan SSR, Azer. Neft. Khoz., 1983, No. 4, pages 40-43 attempted to prepare synthetic lubricants by oligomerizing long-chain (Cs-C14) olefins using non-hazardous and non-polluting acidic clays comprising sulphuric and hydrochloric acid-activated bentonites from the Azerbaidzhan SSR. They concluded that "it was not possible to prepare viscous or high-viscosity oils by olefin polymerization over an aluminosilicate catalyst" and that "hydrogen redistribution reactions predominate with formation of aromatic hydrocarbon, coke, and paraffinic hydrocarbon". US-A-4531014, on the other hand, discloses the use of Wyoming bentonite to oligomerize shorter-chain olefins, but this process, like that of Kuliev et al., does not provide a product high in dimer, trimer and tetramer, and low in disproportionation products.

Our prior Application (P23492) 91302130.9 discloses that it is possible to prepare synthetic lubricant base stocks in good yield by oligomerizing long-chain olefins using certain acidic montmorillonite clay catalysts. We have found that a high conversion of long-chain olefin into dimer, trimer and tetramer may be obtained, with formation of very little concomitant hydrogen redistribution by-product, by using an acidic calcium montmorillonite clay having a moisture content of up to 20 wt.%, a residual acidity of 3 to 30mg KOH/g (when titrated to a phenolphthalein end point), and a surface area of 300 M²/g or more. In addition to being excellent catalysts, these clays are non-hazardous and non-polluting.

We have now discovered that the viscosity (and in some instances the pour point) of base stocks prepared in this manner may be improved by co-reacting a major amount of long-chain linear olefin and minor amount of certain aromatic compounds (i.e. in a mole ratio of about 3:1 or greater), for example anisole, diphenyl ether and/or diphenyl. The resulting mixtures of oligomers and alkylated anisoles, phenyl ethers and/or alkylated diphenyls exhibit a good viscosity and, with the alkylated diphenyl ethers and a diphenyls, a pour point substantially lower than that observed in base stocks comprising the olefin oligomers alone. The incorporation of an ether linkage (in the case of anisole and diphenyl ether) serves to increase the additive solubility of the resulting base stocks as well. The oligomers and alkylated anisoles, alkylated diphenyl ethers and/or alkylated diphenyls may be hydrogenated (to alkanes and alkylated cyclohexyl ethers and/or alkylated dicyclohexanes) to enhance their oxidative stability. US-A-4480142 discloses a process for preparing alkylated polycyclic aromatics by contacting the aromatic compound with an alpha olefin in a mole ratio of olefin to aromatic of up to 2.5:1. An acidic montmorillonite clay is used to catalyze the reaction.

One embodiment of this invention provides a synthetic lubricant base stock comprising oligomers prepared from an olefin composition comprising a linear olefin having from 10 to 24 carbon atoms, which base stock additionally contains an alkyl-substituted diphenyl, diphenyl ether or anisole having the formula:
wherein R¹ is a group of the formula
and where R², R³, R⁴, R⁵, R⁶ and R⁷ are each H or an alkyl group having 1 to 24 carbon atoms, provided that at least one of R², R³, R⁴, R⁵, R⁶ and R⁷ is an alkyl group containing from 10 to 24 carbon atoms, R11 is an alkyl group having 1 to 10 carbon atoms; R² is an alkyl group having 10 to 24 carbon atoms; and R³ and R⁴ are each H or an alkyl group having up to 10 carbon atoms.

An embodiment of this invention provides such a composition which additionally contains an alkyl-substituted aromatic or cycloaliphatic compound having the formula:
and where R² to R⁷ and R¹¹ to R¹⁴ have the meanings given above.

The linear olefins can comprise alpha-olefins, internal olefins or a mixture thereof.

In another embodiment the olefin composition comprises said linear olefins and up to 20 weight % of propylene or of 1,3-diisopropenyl benzene or alpha-methyl styrene.

Alternatively the olefin composition can comprise said linear olefins and a vinylidene olefin having 10 to 24 carbon atoms, e.g. 5 to 40 weight % of the vinylidene olefin.

The invention also provides a process for producing a synthetic lubricant base stock as defined above by contacting the olefin composition with an acidic montmorillonite clay in the presence of an alkyl-substituted diphenyl, diphenyl ether or anisole having the formula
wherein R¹ is a group of the formula
where R² to R⁷ have the meanings given above provided at least one of R² to R⁷ is hydrogen, R11 is alkyl having 1 to 10 carbon atoms, R¹² is hydrogen, and R¹³ and R¹⁴ are each hydrogen or alkyl ethers and/or alkylated diphenyls contained in the mixture may then be hydrogenated, to obtain a mixture of reduced oligomers and alkylated cyclohexyl ethers and/or alkylated dicyclohexanes. Preferably, the resulting base stocks contain from 1 to 50 wt.% of alkylated cyclohexyl ethers and/or alkylated dicyclohexanes. More preferably, the resulting base stocks contain from 5 to 25 wt.% of alkylated cyclohexyl ethers and/or alkylated diclohexanes. Optionally, one skilled in the art may use those hydrogenation conditions which will reduce only the oligomers, to obtain a mixture comprising reduced oligomers and alkylated phenyl ethers and/or alkylated diphenyls. One skilled in the art also may find it desirable to use those hydrogenation conditions which will reduce the oligomers and a portion of the alkylated phenyl ethers and/or alkylated diphenyls, to obtain a mixture comprising reduced oligomers, alkylated phenyl ethers and/or alkylated diphenyls and alkylated cyclohexyl ethers and/or alkylated dicyclohexanes. Compounds with one aromatic ring and one cyclohexyl (reduced) ring may be prepared and included as well.

According to another embodiment, the viscosity of the base stocks is improved when the starting materials comprise a mixture of long-chain linear olefin and anisole, preferably from 1 to 40 wt.% of anisole (i.e. a weight ratio of anisole to linear olefin of 1:99 to 2:3). More preferably, the mixture of long-chain linear olefin and anisole contains from 5 to 25 wt.% of anisole (i.e. a weight ratio of anisole to linear olefin of 1:20 to 1:4). It is especially preferred that the mixture of long-chain linear olefin and anisole contain about 20 wt.% anisole (i.e. a weight ratio of anisole to linear olefin of about 1:5). Co-reacting the anisole and linear olefin feed produces a mixture of olefin oligomers and alkylated anisoles. Optionally, the double bonds present in the oligomers and alkylated anisoles contained in the mixture may then be hydrogenated, to obtain a mixture of reduced oligomers and alkylated methoxycyclohexanes. Preferably, the resulting base stocks contain from 1 to 80 wt.% alkylated methoxycyclohexane. More preferably, the resulting base stocks contain from 5 to 40 wt.% of alkylated methoxycyclohexane. having 1 to 10 carbon atoms.

The clay can optionally be activated with a Lewis acid.

The alkylation-oligomerization product of this reaction can be completely or partially hydrogenated.

Our prior Application (P23492) 91302130.9 indicates that synthetic lubricant base stocks may be prepared in good yield by oligomerizing long-chain linear olefins using certain acidic montmorillonite clay catalysts. We have now found that the viscosity (and in certain instances, the pour point) of these base stocks can be improved when the starting materials comprise a mixture of a major amount of a long-chain linear olefin and a minor amount of certain aromatic compounds, for example, anisole, phenyl ether and/or diphenyl. As used herein, the phrase "phenyl ether and/or diphenyl" indicates that the mixture may contain one of the following: (1) phenyl ether and no diphenyl; (2) diphenyl and no phenyl ether; or (3) both phenyl ether and diphenyl in a ratio of phenyl ether to diphenyl of 1:99 to 99:1. The use of "and/or" in connection with other components of mixtures described herein is to be interpreted similarly, indicating the presence of either (or, if three or more, any) component without the other(s), or both (or, if three or more, some or all).

The starting material used to prepare the base stocks of the present invention comprise a mixture containing a long-chain linear olefin and certain aromatic compounds in a mole ratio of olefin to aromatic compound of 3:1 or greater. Co-reacting a major amount of linear olefin feed with a minor amount of anisole, phenyl ether and/or diphenyl produces a mixture of olefin oligomers with alkylated anisoles, alkylated phenyl ethers and/or alkylated diphenyls. Preferably, the resulting base stocks contain from 1 to 50 wt. % of alkylated phenyl ethers and/or alkylated diphenyls. More preferably, the resulting base stocks contain from 5 to 25 wt.% of alkylated phenyl ethers and/or alkylated diphenyls. Optionally, the double bonds present in the oligomers and alkylated phenyl One skilled in the art may find it desirable to use those hydrogenation conditions which will reduce only the oligomers, to obtain a mixture comprising reduced oligomers and alkylated anisoles. One skilled in the art also may find it desirable to use hydrogenation conditions which will reduce the oligomers and a portion of the alkylated anisoles, to obtain a mixture comprising reduced oligomers, alkylated anisoles and alkylated methoxycyclohexanes.

Olefin monomer feed stocks useful in the present invention include compounds comprising (1) alpha-olefins having the formula R"CH = CH₂, where R" is an alkyl radical of 8 to 22 carbon atoms, and (2) internal olefins having the formula RCH = CHR', where P and R' are the same or different alkyl radicals of 1 to 20 carbon atoms, provided that the total number of carbon atoms in any one olefin shall be within the range of 10 to 24, inclusive. A preferred range for the total number of carbon atoms in any one olefin molecule is 12 to 18, inclusive, with any especially preferred range being 13 to 16, inclusive. Mixtures of internal and alpha-olefins may be used, as well as mixtures of olefins having different numbers of carbon atoms, provided that the total number of carbon atoms in any one olefin shall be within the range of 10 to 24, inclusive. The alpha and internal-olefins useful in the present invention may abe obtained by processes well-known to those skilled in the art and are commercially available. It is also possible to co-oligomerize additional unsaturated hydrocarbons with the linear olefins. Examples include propylene, diisopropenyl benzene, alpha-methyl styrene and vinylidine olefins. For more information, reference may be made to our prior Application (P23492) 91302130.9.

Anisole, also known as methyl phenyl ether, may be obtained by processes well-known to those skilled in the art and is commercially available. While anisole is preferred in this embodiment of the present invention, acceptable substitutes for anisole include those compounds having the following structure:
where R11 is an alkyl group having 1 to 10 carbon atoms; R¹² is hydrogen. and R¹³ amd R14 are each hydrogen or an alkyl group having 1 to 10 carbon atoms.

Diphenyl ether and diphenyl may be obtained by processes well-known to those skilled in the art and are commercially available. While diphenyl ether (C₆H₅OC₆H₅) and diphenyl (C₆H₅C₆H₅) are preferred in this embodiment of the present invention, acceptable substitutes for diphenyl ether and diphenyl include those aromatic compounds having the following structures:
and where R², R³, R⁴, R⁵, R⁶, and R⁷ are each hydrogen or an alkyl group having from 1 to 24 carbon atoms. It is preferred that R², R³, R⁴, R⁵, R⁶, and R⁷ contain no more than 10 carbon atoms. At least one of ^{R2, R3, R4,} R^{5,} R⁶, or R⁷ is H.

Oligomerization of linear olefins may be represented by the following general equation:
where n represents moles of monomer and m represents the number of carbon atoms in the monomer. Thus, oligomerization of 1-decene may be represented as follows:

The reactions occur sequentially. Initially, olefin monomer reacts with olefin monomer to form dimers. The dimers that are formed then react with additional olefin monomer to form trimers, and so on. This results in an oligomer product distribution that varies with reaction time. As the reaction time increases, the olefin monomer conversion increases, and the selectivities for the heavier oligomers increase. Generally, each resulting oligomer contain one double bond.

The mono-alkylation of phenyl ether, anisole and diphenyl by a linear olefin may be represented respectively as follows:
where m = the number of carbon atoms in the olefin monomer. Depending on the mole ratio of linear olefin to phenyl ether, anisole, and/or diphenyl and on the reaction conditions, poly-alkylation of the phenyl ether anisole and/or diphenyl also will occur. The alkylation of phenyl ether, anisole and/or diphenyl by linear olefin feed occurs concurrently with the oligomerization of the olefin feed. Thus, the co-reaction results in a mixture of oligomers (dimers, trimers, tetramers, etc) and alkylated phenyl ether, alkylated anisole, and/or alkylated diphenyls, including mono-, di-, and tri- alkylated phenyl ether -anisole, and/or -diphenyl. The number of carbon atoms in the alkyl groups of the alkylated phenyl ether, anisole, and/or alkylated diphenyls will correspond to the number of carbon atoms in the linear olefin feed. Thus, the alkyl groups of the alkylated phenyl ether, anisole, and/or alkylated diphenyls will have from 10 to 24 carbon atoms.

The catalysts useful to effect these reactions are examples of silica-alumina clays, also called aluminosilicates. Silica-alumina clays primarily are composed of silicon, aluminium and oxygen, with minor amounts of magnesium and iron in some instances. Variations in the ratios of these constituents, and in their crystal lattice configurations, result in some fifty separate clays, each with its own characteristic properties.

One class of silica-alumina clays comprises smectite clays, which have a small particle size and unusual intercalation properties which afford them a high surface area. Smectites comprise layered sheets of octahedral sites between sheets of tetrahedral sites, where the distance between the layers can be adjusted by swelling, using an appropriate solvent. Three-layered sheet-type smectites include montmorillonites. The montmorillonites structure may be represented by the following formula
where M represents the intermellar (balancing) cations, normally sodium or lithium; and x, y and n are numbers.

Montmorillonite clays may be acid-activated by such mineral acids as sulphuric acid and hydrochloric acid. Mineral acids activate montmorillonites by attacking and solubilizing structural cations in the octahedral layers. This opens up the clay structure and increases surface area. These acid-treated clays act as strong Bronsted acids. We have discovered that certain acid-treated montmorillonite clay catalysts are particularly effective for preparing synthetic lubricant base stocks in good yield by oligomerizing long-chain olefins. These clays are acidic calcium montmorillonite clays having a moisture content of up to 20 wt.%, a residual acidity of 3 to 30mg KOH/g (when titrated to a phenolphthalein end point), and a surface area of 300 M²/g or more. Illustrative examples include Filtrol grade 24, having a moisture content of 12 wt.%, a residual acidity of 8.5 mg KOH/g and a surface area of 425 M²/g; Filtrol grade 124, having a moisture content of 2 wt%, residual acidity of 7.0 mg KOH/g, and a surface area of 400 M²/g; Filtrol grade 13, having a moisture content of 16 wt.%, a residual acidity of 15 mg KOH/g, and a surface area of 300 M²/g; Filtrol grade 113, having a moisture content of 4 wt.%, a residual acidity of 10 mg KOH/g, and a surface area of 300 M²/g; and Filtrol grade 224, having virtually no moisture, and having a residual acidity of 3.0 mg KOH/g, and a surface area of 350 M²/g.

Preferably, the clay catalyst is activated by heat treatment before running the co-reactions. We have found that heat treatment of the catalyst before running an oligomerization reaction causes the catalyst to be more active and to produce a higher olefin conversion. Additionally, clays heat treated in this manner are more stable, remaining active for a long period during a reaction. The clays may be heat treated at temperatures of 50 to 400 C, with or without the use of a vacuum. A more preferred temperature range is 50 to 300 C. Optionally, an inert gas may be used during heat treatment as well. Preferably, the clay should be heat treated under conditions and for a length of time which will reduce the water content of the clay to approximately 1 wt.% or less. The clay may also be activated by a Lewis acid, see our prior Application (P23492) 91302130.9.

The oligomerization and alkylation co-reactions may be carried out in a stirred slurry reactor or in a fixed bed continuous flow reactor. The catalyst concentration should be sufficient to provide the desired catalytic effect. The temperatures at which the oligomerization and alkylation may be performed are generally from 50 to 300 C, with the preferred range being from 150 to 180°C. The reactions may be run at pressures of from 0.1 to 7 MPa (0 to 1000 psig).

Preferably, following the oligomerization and alkylation co-reactions, the partially unsaturated oligomers are completely reduced via catalytic hydrogenation. Depending on the hydrogenation conditions employed, the alkylated phenyl ethers, alkylated anisoles, and/or alkylated diphenyls may be completely or partially reduced as well, or, if desired, may remain in the aromatic form; preferably, they are completely reduced. Hydrogenation of the oligomers and the alkylated anisole, alkylated phenyl ether and/or alkylated diphenyls improves their thermal stability and helps prevent oxidative degradation during use of the mixture as a lubricant. The hydrogenation reaction for 1-decene oligomers may be represented as follows:
where n represents moles of monomer used to form the oligomer. The complete hydrogenation of a mono-alkylated phenyl ether, mono-alkylated anisole, or mono-alkylated diphenyl may be represented respectively, as follows:

Hydrogenation processes known to those skilled in the art may be used. A number of metal catalysts are suitable for promoting the hydrogenation reaction, including nickel, platinum, palladium, copper, and Raney nickel. These metals may be supported on a variety of porous materials, such as kieselguhr, alumina, or charcoal. A particularly preferred catalyst for this hydrogenation is a nickel-copper-chromia catalyst described in US-A-3152998 other known hydrogenation procedures are disclosed in US-A-4045508, -4013736, -3997621 and -3997622. To reduce the double bonds of both the oligomers and alkylated anisoles, alkylated phenyl ethers and/or alkylated diphenyls, the hydrogenation conditions described in the examples below may be employed. To reduce only the oligomers, less vigorous conditions should be used, such as the following: using a 0.5% palladium on alumina catalyst (10 wt.% based on charge), pressurize to 3.5 MPa (500 psig) with hydrogen and heat to 90 C; re-pressurize to 7MPa (1000 psig) with hydrogen as needed, for 4 hours.

Unreacted monomer and anisole, phenyl ether and/or diphenyl may be removed either before or after hydrogenation Optionally, unreacted monomer and anisole, phenyl ether and/or diphenyl may be stripped from the oligomers/alkylated phenyl ethers, alkylated anisoles, and/or alkylated diphenyls before hydrogenation and recycled to the catalyst bed for co-reaction. The removal or recycle of unreacted monomer and anisole, phenyl ether and/or diphenyl or, if after hydrogenation, the removal of non-oligomerized alkane and non-alkylated cyclohexyl ethers and/or non-alkylated dicyclohexanes, should be conducted under mild conditions using vacuum distillation procedures known to those skilled in the art. Distillation at temperatures exceeding 250 C may cause the oligomers to break down in some fashion and come off as volatiles. Preferably, therefore, the reboiler or pot temperature should be kept at or below 255 C most preferably at or below 180C. Procedures known by those skilled in the art to be alternatives to vacuum distillation also may be employed to separate unreacted components from the mixture.

While it is known to include a distillation step after the hydrogenation procedure to obtain products having various 100°C viscosities, it is preferred in the method of the present invention that no further distillation (beyond removal of any unreacted monomer/linear alkane and phenyl ether/cyclohexyl ether and/or diphenyl/alkylated dicyclohexane) should be conducted. Thus, the method of this invention does not require the costly, customary distillation step, yet, surprisingly, produces a synthetic lubricant component that has excellent properties and that performs in a superior fashion. However, in some contexts, one skilled in the art may find subsequent distillation useful in the practice of this invention.

The invention will be further illustrated by the following Examples:

### EXAMPLES

### Procedure

Reactants and clay catalyst were charged to a three-necked flask equipped with an overhead stirrer, heating mantle, and a nitrogen purge. The mixture was vigorously stirred and heated at the desired temperature for the desired period of time. At the end of the reaction, the mixture was cooled to ambient temperature and filtered with suction. Percentage olefin conversion and dimer/trimer ratio were determined by liquid chromatography and recorded in the Tables below.

An autoclave was charged with nickel catalyst (5 wt.%) and the mixture prepared above. The autoclave was then sealed and flushed three or four times with hydrogen. The autoclave was then pressurized to 7MPa (1000 psig) with hydrogen and heated to 200 C. The mixture was stirred at this temperature for 4.0 hours. The autoclave was repressurized to 14.9MPa (2000 psig) as needed. The mixture was then cooled to ambient temperature and filtered. Unreacted monomer was then removed from the filtrate under vacuum of approximated 133Pa (1 mm Hg). The properties shown in the Tables below were determined on the "stripped" bottoms product.

## Claims

1. A synthetic lubricant base stock comprising oligomers prepared from an olefin composition comprising a linear olefin having from 10 to 24 carbon atoms, characterized in that it additionally contains an alkyl-substituted diphenyl, diphenyl ether or anisole having the formula:
wherein R¹ is a group of the formula
and where R², R³, R⁴, R⁵, R⁶ and R⁷ are each H or an alkyl group having 1 to 24 carbon atoms, provided that at least one of R², R³, R⁴, R⁵, R⁶ and R⁷ is an alkyl group containing from 10 to 24 carbon atoms, R¹¹ is an alkyl group having 1 to 10 carbon atoms; R² is an alkyl group having 10 to 24 carbon atoms; and R³ and R⁴ are each H or an alkyl group having up to 10 carbon atoms.

2. A synthetic lubricant base stock comprising reduced oligomers prepared from an olefin composition comprising a linear olefin having from 10 to 24 carbon atoms, characterized in that it additionally contains an alkyl-substituted aromatic or cycloaliphatic compound having the formula
and where R² to R⁷ and R¹¹ to R¹⁴ have the meanings given in Claim 1.

3. A synthetic lubricant base stock according to Claim 1 or 2 characterized in that the linear olefins comprise alpha-olefins, internal olefins or a mixture thereof.

4. A synthetic lubricant base stock according to any one of Claims 1 to 3 characterized in that the olefin composition comprises said linear olefins and up to 20 weight % of propylene.

5. A synthetic lubricant base stock according to any one of Claims 1 to 3 characterized in that the olefin composition comprises said linear olefins and up to 20 weight % of 1,3-diisopropenyl benzene or alpha-methylstyrene.

6. A synthetic lubricant base stock according to any one of Claims 1 to 3 characterized in that the olefin composition comprises said linear olefins and a vinylidene olefin having 10 to 24 carbon atoms.

7. A synthetic lubricant base stock according to Claim 6 characterized in that the olefin composition contains 5 to 40 weight % of the vinylidene olefin.

8. A process for producing a synthetic lubricant base stock according to any one of Claims 1 and 3 to 7 by contacting the olefin composition with an acidic montmorillonite clay characterized in that the olefin composition is co-reacted with an alkyl-substituted diphenyl, diphenyl ether or anisole having the formula
wherein R¹ is a group of the formula
where R² to R⁷ have the meanings given in Claim 1, provided at least one of R² to R⁷ is hydrogen, R¹¹ is alkyl having 1 to 10 carbon atoms, R¹² is hydrogen, and R¹³ and R14 are each hydrogen or alkyl having 1 to 10 carbon atoms.

9. A process according to Claim 8 characterized in that the clay is activated with a Lewis acid.

10. A process for producing a synthetic lubricant base stock according to Claim 2 characterized by completely or partially hydrogenating a synthetic lubricant base stock according to Claim 1.
